# EUROPEAN PATENT SPECIFICATION

(11) **EP 1 680 537 B1**
(45) Date of publication and mention of the grant of the patent: **02.10.2013**
(21) Application number: 03796987.0
(22) Date of filing: 12.12.2003
(51) Int. Cl.: D01F 6/96, D01F 8/16, D06M 15/37, H01B 1/12

(54) **DURABLE HIGHLY CONDUCTIVE SYNTHETIC FABRIC CONSTRUCTION**
DAUERHAFTE HOCHLEITFÄHIGE SYNTHETISCHE STOFFKONSTRUKTION
TISSU SYNTHETIQUE DURABLE FORTEMENT CONDUCTEUR

(30) Priority: 03.11.2003 US 699997
(43) Date of publication of application: 19.07.2006
(73) Proprietor: ALBANY INTERNATIONAL CORP., Rochester, NH 03867 (US)
(72) Inventor: LEVINE, Mark, J., Hendersonville, TN 37075 (US); O'CONNOR, Joseph, G., Hopedale, MA 01747 (US); DITARANTO, Frank, Norton, MA 02766 (US); TONEY, Crayton, Gregory, Wrentham, MA 02093 (US); LUO, Shuiyuan, Syracuse, NY 13205 (US)
(74) Representative: Bugnion Genève
(86) International application number: PCT/US2003/039623
(87) International publication number: WO 2005/047576

(56) References cited:
- EP-A- 1 091 026
- WO-A-00/75406
- WO-A-99/15725
- "NEOSTAT 2001 - The new solution for your Reicofil line ...", COFPA
- S. Adanur: "Asten PAPER MACHINE CLOTHING", Technomic, Lancaster pages pages202-358-361,

## Description

### Field of the Invention

The present invention is directed towards a conductive fabric construction, particularly one that effectively dissipates static charge whilst also having desirable physical properties.

### Background of the Invention

Heretofore, conductive fabrics useful for, as an example, dissipation of static electricity, have incorporated monofilaments with high loadings of conductive materials, such as carbon black or metallic particulate. Typically, these conductive materials are either dispersed within a base polymer, such as polyethylene terephthalate and polyamide, or incorporated in polymeric coatings which are deposited over oriented monofilaments.

There are several limitations associated with these prior art methods. First, the conductivity of the loaded monofilaments is only in the range of 10⁻⁴ - 10⁻⁷ S/cm, which is the bare minimum needed for effective dissipation of static charge. Unfortunately, this drawback limits the fabric design options, and also impairs fabric performance. A second disadvantage is that, in the case of fully filled products, there is a compromise of monofilament physical properties, such as modulus, tenacity and elongation. This is due to the high level of contamination caused by compounding levels greater than twenty percent of the conductive filler. This loss of physical properties, again, restricts the options for fabric design and negatively impacts fabric performance. A further shortcoming associated with prior art conductive fabrics is that highly loaded carbon -based coatings exhibit both poor abrasion and inferior adhesion properties. Consequently, the fabric's durability along with its dissipation properties both suffer.

Other prior art conductive fabrics incorporate conductive coatings, metallic wire constructions, or combination designs incorporating metallic additive fibers within a synthetic structure. There are, however, drawbacks also associated with these fabrics. For example, while these prior designs may dissipate static charge, it is noted that structures with metallic wires are difficult to manufacture. A further disadvantage is that metal-based fabrics are easily damaged, and in particular, incur unwanted dents and creases during use. Prior art coated designs, on the other hand, have suffered from a lack of durability and also interfere with the permeability of open mesh structures.

The incorporation of electrically conductive polymers into fabrics presents a potential solution to the forgoing problems. In this connection, conductive polymers are available either as the polymer itself or a doped form of a conjugated polymer. Additionally, conductivities as high as 30-35 x 10³ S/cm have been achieved using these polymers, which is only an order of magnitude below the conductivity of copper. However, in addition to being sufficiently conductive, the polymer must also be stable in air at use temperature and so retain its conductivity over time. Also, the conductive polymer material must be processable, and have sufficient mechanical properties for a particular application.

### Summary Of The Invention

It is therefore a principal object of the invention to incorporate conductive polymers into forms that can be manufactured into durable fabric constructions.

This and other objects and advantages are provided by the present invention. In this regard, the present invention is directed towards a durable, highly conductive, synthetic fabric construction. Advantageously, the invention involves using functional filaments containing conductive polymer material. As a result, synthetic fabrics comprised of these conductive filaments have static dissipation properties previously available only in metal-based fabrics, whilst also having physical properties comparable to non-conductive fabrics. Consequently, the inventive fabric construction resists the denting and creasing associated with metallic fabric designs.

### Brief Description of the Drawing

Thus by the present invention, its objects and advantages will be realized the description of which should be taken in conjunction with the drawing wherein:
Figure 1 is a cross sectional view of a lobed monofilament coated with an electrically conductive polymer, according to the teachings of the present invention.

### Detailed Description of the Preferred Embodiments

A preferred embodiment of the present invention will be described in the context of engineered fabrics, such as fabrics used in making non-woven textiles in the airlaid, meltblown and/or spunbonding processes. However, it should be noted that the invention is also applicable to other industrial fabrics used in any "dry" applications where the dissipation of static electricity is required, for instance, through the belting media. Fabric constructions include woven, nonwoven, spiral-link, MD or CD yarn arrays, knitted fabric, extruded mesh, and spiral wound strips of woven and nonwoven materials. These fabrics may comprise monofilament, plied monofilament, multifilament or plied multifilament synthetic yarns, and may be single-layered, multi-layered or laminated.

Turning now more particularly to the drawing, the invention provides for fabrics comprising, as shown in Figure 1 (cross sectional view), functional filament(s) 10 containing electrically conductive polymer material 14. Thus, whereas conductive polymers by themselves generally lack the strength to be formed into load bearing filaments 10, the invention incorporates these conductive materials 14 as either blends or coatings in conjunction with polymeric materials that can be oriented to achieve physical properties needed to form durable fabric structures. Advantageously, fabrics incorporating at least five percent of these conductive filaments 10 have static dissipation properties equivalent to, and previously available only in, metal-based fabrics, whilst possessing physical properties equivalent to non-conductive fabrics. Consequently, fabrics with these filaments 10 resist the denting and creasing heretofore associated with metal designs.

In particular, the invention incorporates the conductive polymer 14 as blends into monofilaments 12 having sufficient thermal stability. Alternatively, the invention envisions bicomponent fibers containing the conductive polymer 14 and produced using melt extrusion. As a further option, Figure 1 illustrates a preferred embodiment wherein the conductive polymer 14 is applied to the monofilament 12 as a coating. Techniques include, for example, dip coating, spraying from solutions, dispersions over oriented monofilaments, thermal spraying, or other means suitable for the purpose. Notably, there is at least one class of conductive polymers, polyanilines, from which filaments have been produced with high conductivities and physical properties comparable to polyamides. Accordingly, the invention provides for using these conductive filaments directly in fabrics.

The embodiment shown cross sectionally in Figure 1 provides for coating a lobed monofilament 12 with the conductive polymer material 14. Advantageously, this increases the monofilament's conductivity beyond 10⁻³ S/cm (preferably beyond 10³ S/cm), whilst maintaining the monofilament's physical and tribological properties. As a further benefit, the surface 16 of the monofilament 12 has a plurality of C-shaped grooves 18 running along the length thereof, and these grooves 18 may be formed during the extrusion of the monofilament 12. Consequently, a mechanical interlock forms between the monofilament 12 and the polymer material 14 filling the grooves 18. This configuration thus reduces the need for adhesion of the polymer 14 to the monofilament 12. As a further advantage, this arrangement allows continued exposure of the highly conductive polymer 14 to the surface 16 even as the monofilament 12 wears, whilst also shielding and protecting the polymer material 14. In addition the protective positioning of the conductive polymer 14 reduces the impact of the polymer's lesser abrasion resistance and physical properties. Incidentally, in addition to the circular shape shown in Figure 1, the monofilament 12 can obviously also have a non-circular cross sectional shape such as rectangular, square, trapezoidal, oblong, oval, conical, star-shaped, or other non-circular shapes suitable for the purpose.

A yet further benefit of the invention is that the weight percent composition of the conductive polymer 14 can be only ten percent or less of the filament 10. This keeps fabric production costs down while providing effective dissipation of the static charge. In this connection, classes of conductive polymers 14 that can be used include: polyacetylene (PA), polythiophene (PT), poly3alkyl-thiophene) (P3AT), polypyrrole (Ppy), poly-isothianaphthene (PITN), poly(ethylene dioxythiophene (PEDOT), alkoxy-substituted poly(paraphenylene vinylene) (PPV), poly(para-phenylene vinylene) (PPV), poly(2,5-dialkoxy-para-phenylene), poly(para-phenylene) (PPP), ladder-type poly(paraphenylene) (LPPP), poly(para-phenylene) sulfide (PPS), polyheptadiyne(PHT), poly(3-hexyl thiophene) (P3HT), polyaniline (PANI).

Thus by the present invention its objects and advantages are realized, and although preferred embodiments have been disclosed and described in detail herein, its scope and objects should not be limited thereby; rather its scope should be determined by that of the appended claims.

## Claims

1. A conductive engineered industrial belting media suitable for making nonwoven textiles in the airlaid, meltblown or spunbonding processes comprising a plurality of load-bearing oriented polymeric filaments (10) having one or more shaped grooves (18) formed on the surface (16) and running along the length of the filaments (10), wherein each filament (10) includes electrically conductive polymer material (14) incorporated as either a blend or a coating that substantially fills the shaped grooves (18), wherein the cross-section of each shaped groove (18) presents a shape that provides a mechanical interlock between a monofilament (12) and the conductive polymer (14), said conductive belting media having static dissipation properties comparable to metal-based belting media whilst being resistant to dents and creases and wherein the one or more shaped grooves (18) allow for continued exposure of the conductive polymer (14) to the filament surface (16) as the monofilament (12) wears so that the filament (10) retains its conductivity.

2. The industrial belting media in accordance with claim 1, wherein the functional filaments (10) constitute between five and one hundred percent of the fabric.

3. The industrial belting media in accordance with claim 1, wherein the fabric has static dissipation properties of metal-based fabrics whilst also having physical properties comparable to non-conductive synthetic fabrics.

4. The industrial belting media in accordance with claim 3, wherein said physical properties include one of modulus, tenacity, strength, adhesion, abrasion resistance, and durability.

5. The industrial belting media in accordance with claim 1, wherein the filament (10) comprises conductive polymer material (14) blended with polymeric materials that can be oriented.

6. The industrial belting media in accordance with claim 1, wherein the filament (10) is a bicomponent fiber containing conductive polymer material (14) and formed by melt extrusion.

7. The industrial belting media in accordance with claim 1, wherein the filament (10) comprises an oriented structure coated with conductive polymer material (14).

8. The industrial belting media in accordance with claim 7, wherein the conductive polymer (14) is applied by one of dip coating, spraying from solutions, dispersion over the filament, and thermal spraying.

9. The industrial belting media in accordance with claim 1, wherein the filament (10) comprises conductive polymer material (14) selected from the class of polyanilines.

10. The industrial belting media in accordance with claim 9, wherein said polyaniline filament has physical properties of a polyamide filament.

11. The industrial belting media in accordance with claim 1, wherein the filament (10) is a lobed monofilament (12) coated with conductive polymer material (14).

12. The industrial belting media in accordance with claim 11, wherein the coating (14) has a conductivity, minimally greater than 10⁻³ S/cm, whilst maintaining the physical and tribological properties of the core monofilament (12).

13. The industrial belting media in accordance with claim 11, wherein the shape of the one or more shaped grooves (18) includes C-shaped grooves that provide a mechanical interlock between the monofilament and the conductive polymer (14) filling the grooves (18).

14. The industrial belting media in accordance with claim 13, wherein the interlock provided by the C-shaped grooves (18) reduces a need for adhesion of the conductive polymer (14) to the monofilament (12) by providing the mechanical interlock between the monofilament and the conductive polymer filling the grooves (18).

15. The industrial belting media in accordance with claim 13, wherein positioning of the conductive polymer (14) in the C-shaped grooves (18) shields the polymer and reduces the impact of its lesser abrasion resistance and physical properties.

16. The industrial belting media in accordance with claim 11, wherein the weight composition of the conductive material (14) is ten percent or less of the total weight of the coated monofilament (12).

17. The industrial belting media in accordance with claim 1, wherein the fabric is single-layered or multi-layered, or laminated.

18. The industrial belting media in accordance with claim 1, wherein the industrial belting media is one of woven, nonwoven, spiral-link, MD or CD yarn arrays, knitted fabric, extruded mesh, and spiral wound strips of woven and nonwoven materials.

19. The industrial belting media in accordance with claim 1, wherein the fabric is suitable for a dry application in which static dissipation is required through the belting media.

20. The industrial belting media in accordance with claim 1, wherein the conductive polymer (14) is one of polyacetylene, polythiophene, poly3alkyl-thiophene, polypyrrole, poly-isothianaphthene, polyethylene dioxythiophene, alkoxy-substituted poly(para-phenylene vinylene), poly(para-phenylene vinylene), poly(2,5-dialkoxypara-phenylene), poly(paraphenylene), ladder-type poly(paraphenylene), poly(para-phenylene) sulfide, polyheptadiyne, and poly(3-hexyl thiophene).

21. The industrial belting media in accordance with claim 11, wherein the coating (14) has a conductivity greater than 10³ S/cm, whilst maintaining the physical and tribological properties of the core monofilament (12).

22. The industrial belting media in accordance with claim 1, wherein the industrial belting media is laminated.

23. The industrial belting media in accordance with claim 18, wherein the spiral wound strips are woven or nonwoven materials comprising yarns including monofilaments, plied monofilaments, multifilaments, plied multifilaments and staple fibers.

24. The industrial belting media in accordance with claim 1, wherein the monofilament (12) has a non-circular cross sectional shape.

25. The industrial belting media in accordance with claim 24, wherein the monofilament (12) has the non-circular cross sectional shape selected from the group of: rectangular, square, trapezoidal, oblong, oval, conical or star-shaped.

26. The industrial belting media in accordance with claim 25, wherein the monofilament's (12) cross sectional shape is rectangular or square and includes a plurality of grooves.

27. The industrial belting media in accordance with claim 11, wherein the shape of one or more shaped grooves (18) includes a necking that provides a mechanical interlock between the monofilament and the conductive polymer (14) filling the grooves (18).

28. An load bearing polymeric filament (10) suitable for an engineered industrial belting media for making nonwoven textiles in the airlaid, meltblown or spunbonding processes, said polymeric filament (10) having one or more shaped grooves (18) formed on the surface (16) and running along the length of the filament (10), wherein said shaped grooves (18) are substantially filled with electrically conductive polymer material (14) mechanically locked in place and wherein the one or more shaped grooves (18) allow for continued exposure of the conductive polymer (14) to the filament surface (18) as the monofilament (12) wears so that the filament (10) retains its conductivity and wherein the cross-section of each shaped groove (18) presents a shape that provides mechanical interlock between the monofilament (12) and the conductive polymer (14).

29. The filament in accordance with claim 28, wherein the filament (10) comprises conductive polymer material (14) blended with polymeric materials that can be oriented.

30. The filament (10) in accordance with claim 28, wherein the filament (10) is a bicomponent fiber containing conductive polymer material (14) and formed by melt extrusion.

31. The filament (10) in accordance with claim 28, wherein the filament (10) comprises an oriented structure coated with conductive polymer material (14).

32. The filament (10) in accordance with claim 31, wherein the conductive polymer (14) is applied by one of dip coating, spraying from solutions, dispersion over the filament, and thermal spraying.

33. The filament (10) in accordance with claim 28, wherein the filament comprises a conductive polymer material (14) selected from the class of polyanilines.

34. The filament (10) in accordance with claim 33, wherein said polyaniline filament has physical properties of a polyamide filament.

35. The filament (10) in accordance with claim 28, wherein the filament is a lobed monofilament (12) coated with conductive polymer material (14).

36. The filament (10) in accordance with claim 35, wherein the coating (14) has a conductivity, minimally greater than 10³ S/cm, whilst maintaining the physical and tribological properties of the core monofilament.

37. The filament (10) in accordance with claim 35, wherein the shape of the groves (18) includes C-shaped grooves that provide a mechanical interlock between the monofilament (12) and the conductive polymer (14) filling the grooves (18).

38. The filament (10) in accordance with claim 37, wherein the interlock provided by the C-shaped grooves (18) reduces a need for adhesion of the conductive polymer (14) to the monofilament (12) by providing the mechanical interlock between the monofilament (12) and the conductive polymer (14) filling the grooves (18).

39. The filament (10) in accordance with claim 37, wherein positioning of the conductive polymer (14) in the C-shaped grooves (18) shields the polymer (14) and reduces the impact of its lesser abrasion resistance and physical properties.

40. The filament (10) in accordance with claim 35, wherein the weight composition of the conductive material (14) is ten percent or less of the total weight of the coated monofilament (10).

41. The filament (10) in accordance with claim 28, wherein the conductive polymer is one of polyacetylene, polythiophene, poly3alkyl-thiophene, polypyrrole, polyisothia-naphthene, polyethylene dioxythiophene, alkoxy-substituted poly(para-phenylene vinylene), poly(paraphenylene vinylene), poly(2,5-dialkoxy-para-phenylene), poly(para-phenylene), ladder-type poly(para-phenylene), poly(para-phenylene) sulfide, polyheptadiyne, and poly(3-hexyl thiophene).

42. The filament (10) in accordance with claim 35, wherein the coating (14) has a conductivity greater than 10³ S/cm, whilst maintaining the physical and tribological properties of the core monofilament.

43. The filament (10) in accordance with claim 28, wherein the monofilament (12) has a non-circular cross sectional shape.

44. The filament in accordance with claim 43, wherein the monofilament (12) has the non-circular cross sectional shape selected from the group of: rectangular, square, trapezoidal, oblong, oval, conical or star shaped.

45. The filament (10) in accordance with claim 44, wherein the monofilament's (12) non-circular cross sectional shape is rectangular or square and includes a plurality of grooves.

46. The filament (10) in accordance with claim 21, wherein the shape of the one or more shaped grooves (18) includes a necking that provides a mechanical interlock between the monofilament and the conductive polymer (14) filling the grooves (18).

## Patentansprüche

1. Leitfähiges, technisches, industrielles Bandmedium, geeignet zur Herstellung von nicht gewebten Textilien in Luftlege-, Schmelzblas- oder Spinnbindeprozessen, umfassend eine Mehrzahl von tragfähigen orientierten polymeren Filamenten (10) mit einer oder mehreren geformten Rillen (18), die auf der Oberfläche (16) ausgebildet sind und entlang der Länge des Filaments (10) verlaufen, wobei jedes Filament (10) elektrisch leitendes Polymermaterial (14) umfasst, das entweder als eine Mischung oder eine Beschichtung eingearbeitet ist und die geformten Rillen (18) im Wesentlichen füllt, wobei der Querschnitt jeder geformten Rille (18) eine Form darstellt, welche eine mechanische Verriegelung zwischen einem Monofilament (12) und dem leitfähigen Polymer (14) bereitstellt, wobei das leitfähige Bandmedium statische Ableitungseigenschaften besitzt, die mit Bandmedien auf Metallbasis vergleichbar sind, während sie gegen Verbeulungen und Knitterfalten beständig sind, und wobei die eine oder die mehreren Rillen (18) ein kontinuierliches Ausgesetztsein des leitfähigen Polymers (14) an der Filamentoberfläche (16) ermöglichen, wenn sich das Monofilament (12) abnutzt, so dass das Filament (10) eine Leitfähigkeit bewahrt.

2. Industrielles Bandmedium nach Anspruch 1, wobei die funktionellen Filamente (10) zwischen fünf und einhundert Prozent des Gewebes bilden.

3. Industrielles Bandmedium nach Anspruch 1, wobei das Gewebe statische Ableitungseigenschaften von Geweben auf Metallbasis aufweist, während es außerdem physikalische Eigenschaften aufweist, die mit nichtleitenden synthetischen Fasern vergleichbar sind.

4. Industrielles Bandmedium nach Anspruch 3, wobei wobei die physikalischen Eigenschaften eines von Modulus, Zähigkeit, Festigkeit, Haftung, Abriebbeständigkeit und Haltbarkeit umfassen.

5. Industrielles Bandmedium nach Anspruch 1, wobei das Filament (10) leitfähiges Polymermaterial (14) umfasst, das mit polymeren Materialien gemischt ist, die orientiert werden können.

6. Industrielles Bandmedium nach Anspruch 1, wobei das Filament (10) eine Zweikomponentenfaser ist, die leitfähiges Polymermaterial (14) enthält und durch Schmelzextrusion gebildet ist.

7. Industrielles Bandmedium nach Anspruch 1, wobei das Filament (10) eine orientierte Struktur umfasst, die mit leitfähigem Polymermaterial (14) beschichtet ist.

8. Industrielles Bandmedium nach Anspruch 7, wobei das leitfähige Polymer (14) durch eines von Tauchbeschichten, Sprühen von Lösungen, Dispersion über das Filament und thermischem Spritzen aufgetragen ist.

9. Industrielles Bandmedium nach Anspruch 1, wobei das Filament (10) leitfähiges Polymermaterial (14) umfasst, das aus der Klasse von Polyanilinen ausgewählt ist.

10. Industrielles Bandmedium nach Anspruch 9, wobei das Polyanilinfilament physikalische Eigenschaften eines Polyamidfilaments aufweist.

11. Industrielles Bandmedium nach Anspruch 1, wobei das Filament (10) ein profiliertes Monofilament (12) ist, das mit leitfähigem Polymermaterial (14) beschichtet ist.

12. Industrielles Bandmedium nach Anspruch 11, wobei die Beschichtung (14) eine Leitfähigkeit von mindestens über 10⁻³ S/cm bei Aufrechterhaltung der physikalischen und tribologischen Eigenschaften des Kern-Monofilaments (12) aufweist.

13. Industrielles Bandmedium nach Anspruch 11, wobei die Form der einen oder der mehreren Rillen (18) C-förmige Rillen umfasst, die eine mechanische Verriegelung zwischen dem Monofilament und dem die Rillen (18) füllenden leitfähigen Polymer (14) bereitstellen.

14. Industrielles Bandmedium nach Anspruch 13, wobei der Verriegelung, der durch die C-förmigen Rillen (18) bereitgestellt wird, die Notwendigkeit einer Haftung des leitfähigen Polymers (14) am Monofilament (12) durch Bereitstellen der mechanischen Verriegelung zwischen dem Monofilament und dem die Rillen (18) füllenden leitfähigen Polymer reduziert.

15. Industrielles Bandmedium nach Anspruch 13, wobei das Positionieren des leitfähigen Polymers (14) in den C-förmigen Rillen (18) das Polymer abschirmt und die Auswirkung seiner geringeren Abriebbeständigkeit und physikalischen Eigenschaften verringert.

16. Industrielles Bandmedium nach Anspruch 11, wobei die Gewichtszusammensetzung des leitfähigen Materials (14) zehn Prozent oder weniger des Gesamtgewichts des beschichteten Monofilaments (12) beträgt.

17. Industrielles Bandmedium nach Anspruch 1, wobei das Gewebe einlagig, mehrlagig oder laminiert ist.

18. Industrielles Bandmedium nach Anspruch 1, wobei das industrielle Bandmedium eines von gewebt, nicht gewebt, spiralverkettelt, MD- oder CD-Garnanordnungen, gewirktem Stoff, extrudierter Netzware und spiralförmig gewickelten Streifen aus gewebten und nicht gewebten Materialien ist.

19. Industrielles Bandmedium nach Anspruch 1, wobei das Gewebe für eine Trockenanwendung geeignet ist, in welcher statische Ableitung durch das Bandmedium erforderlich ist.

20. Industrielles Bandmedium nach Anspruch 1, wobei das leitfähige Polymer (14) eines von Polyacetylen, Polythiophen, Poly3alkyl-thiophen, Polypyrrol, Polyisothianaphthen, Polyethylendioxythiophen, alkoxysubstituiertem Poly(para-phenylenvinylen), Poly(para-phenylenvinylen), Poly(2,5-dialkoxy-paraphenylen), Poly(paraphenylen), Leiter-Poly(paraphenylen), Poly(para-phenylen)sulfid, Polyheptadiyn, Poly(3-hexylthiophen) ist.

21. Industrielles Bandmedium nach Anspruch 11, wobei die Beschichtung (14) eine Leitfähigkeit von über 10³ S/cm bei Aufrechterhaltung der physikalischen und tribologischen Eigenschaften des Kern-Monofilaments (12) aufweist.

22. Industrielles Bandmedium nach Anspruch 1, wobei das industrielle Bandmedium laminiert ist.

23. Industrielles Bandmedium nach Anspruch 18, wobei die spiralförmig gewickelten Streifen gewebte oder nicht gewebte Materialien sind, die Garne umfassen, die Monofilamente, doublierte Monofilamente, Multifilamente, doublierte Multifilamente und Stapelfasern umfassen.

24. Industrielles Bandmedium nach Anspruch 1, wobei das das Monofilament (12) eine nicht kreisförmige Querschnittsform aufweist.

25. Industrielles Bandmedium nach Anspruch 24, wobei das Monofilament (12) die nicht kreisförmige Querschnittsform aufweist, die aus der Gruppe von Folgendem ausgewählt ist: rechteckig, quadratisch, trapezförmig, länglich, oval, konisch oder sternförmig.

26. Industrielles Bandmedium nach Anspruch 25, wobei die Querschnittsform des Monofilaments (12) rechteckig oder quadratisch ist und eine Mehrzahl von Rillen umfasst.

27. Industrielles Bandmedium nach Anspruch 11, wobei die Form der einen oder der mehreren Rillen (18) eine Querschnittsverringerung umfasst, die eine mechanische Verriegelung zwischen dem Monofilament und dem die Rillen (18) füllenden leitfähigen Polymer (14) bereitstellt.

28. Tragfähiges polymeres Filament (10), geeignet für ein technisches, industrielles Bandmedium zur Herstellung von nicht gewebten Textilien in Luftlege-, Schmelzblas- oder Spinnbindeprozessen, wobei das polymere Filament (10) eine oder mehr geformte Rillen (18) aufweist, die auf der Oberfläche (16) ausgebildet sind und entlang der Länge des Filaments (10) verlaufen, wobei die geformten Rillen (18) im Wesentlichen mit elektrisch leitendem Polymermaterial (14) gefüllt sind, das mechanisch in Stellung verriegelt ist, und wobei die eine oder die mehreren geformten Rillen (18) ein kontinuierliches Ausgesetztsein des leitfähigen Polymers (14) an der Filamentoberfläche (18) ermöglichen, wenn sich das Monofilament (12) abnutzt, so dass das Filament (10) seine Leitfähigkeit bewahrt, und wobei der Querschnitt jeder geformten Rille (18) eine Form darstellt, die eine mechanische Verriegelung zwischen dem Monofilament (12) und dem leitfähigen Polymer (14) bereitstellt.

29. Filament nach Anspruch 28, wobei das Filament (10) leitfähiges Polymermaterial (14) umfasst, das mit polymeren Materialien gemischt ist, die orientiert werden können.

30. Filament (10) nach Anspruch 28, wobei das Filament (10) eine Zweikomponentenfaser ist, die leitfähiges Polymermaterial (14) enthält und durch Schmelzextrusion gebildet ist.

31. Filament (10) nach Anspruch 28, wobei das Filament (10) eine orientierte Struktur umfasst, die mit leitfähigem Polymermaterial (14) beschichtet ist.

32. Filament (10) nach Anspruch 31, wobei das leitfähige Polymer (14) durch eines von Tauchbeschichten, Sprühen von Lösungen, Dispersion über das Filament und thermischem Spritzen aufgetragen ist.

33. Filament (10) nach Anspruch 28, wobei das Filament leitfähiges Polymermaterial (14) umfasst, das aus der Klasse von Polyanilinen ausgewählt ist.

34. Filament (10) nach Anspruch 33, wobei das Polyanilinfilament physikalische Eigenschaften eines Polyamidfilaments aufweist.

35. Filament (10) nach Anspruch 28, wobei das Filament ein profiliertes Monofilament (12) ist, das mit leitfähigem Polymermaterial (14) beschichtet ist.

36. Filament (10) nach Anspruch 35, wobei die Beschichtung (14) eine Leitfähigkeit von mindestens über 10³ S/cm bei Aufrechterhaltung der physikalischen und tribologischen Eigenschaften des Kern-Monofilaments aufweist.

37. Filament (10) nach Anspruch 35, wobei die Form der einen oder der mehreren Rillen (18) C-förmige Rillen umfasst, die eine mechanische Verriegelung zwischen dem Monofilament (12) und dem die Rillen (18) füllenden leitfähigen Polymer (14) bereitstellen.

38. Filament (10) nach Anspruch 37, wobei die Verriegelung, die durch die C-förmigen Rillen (18) bereitgestellt wird, die Notwendigkeit einer Haftung des leitfähigen Polymers (14) am Monofilament (12) durch Bereitstellen der mechanischen Verriegelung zwischen dem Monofilament (12) und dem die Rillen (18) füllenden leitfähigen Polymer (14) reduziert.

39. Filament (10) nach Anspruch 37, wobei das Positionieren des leitfähigen Polymers (14) in den C-förmigen Rillen (18) das Polymer (14) abschirmt und die Auswirkung seiner geringeren Abriebbeständigkeit und physikalischen Eigenschaften verringert.

40. Filament (10) nach Anspruch 35, wobei die Gewichtszusammensetzung des leitfähigen Materials (14) zehn Prozent oder weniger des Gesamtgewichts des beschichteten Monofilaments (10) beträgt.

41. Filament (10) nach Anspruch 28, wobei das leitfähige Polymer (14) eines von Polyacetylen, Polythiophen, Poly3alkyl-thiophen, Polypyrrol, Poly-isothianaphthen, Polyethylendioxythiophen, alkoxysubstituiertem Poly(para-phenylenvinylen), Poly(para-phenylenvinylen), Poly(2,5-dialkoxy-paraphenylen), Poly(para-phenylen), Leiter-Poly(paraphenylen), Poly(para-phenylen)sulfid, Polyheptadiyn, Poly(3-hexylthiophen) ist.

42. Filament (10) nach Anspruch 35, wobei die Beschichtung (14) eine Leitfähigkeit von über 10³ S/cm bei Aufrechterhaltung der physikalischen und tribologischen Eigenschaften des Kern-Monofilaments aufweist.

43. Filament (10) nach Anspruch 28, wobei das Monofilament (12) eine nicht kreisförmige Querschnittsform aufweist.

44. Filament (10) nach Anspruch 43, wobei das Monofilament (12) die nicht kreisförmige Querschnittsform aufweist, die aus der Gruppe von Folgendem ausgewählt ist: rechteckig, quadratisch, trapezförmig, länglich, oval, konisch oder sternförmig.

45. Filament (10) nach Anspruch 44, wobei die nicht kreisförmige Querschnittsform des Monofilaments (12) rechteckig oder quadratisch ist und eine Mehrzahl von Rillen umfasst.

46. Filament (10) nach Anspruch 21, wobei die Form der einen oder der mehreren Rillen (18) eine Querschnittsverringerung umfasst, die eine mechanische Verriegelung zwischen dem Monofilament und dem die Rillen (18) füllenden leitfähigen Polymer (14) bereitstellt.

## Revendications

1. Milieu pour courroie industriel technique conducteur convenant pour la production de textiles non-tissés par des procédés pneumatiques air-laid, de fusion-soufflage et/ou de filage-liage, comprenant une pluralité de filaments polymères orientés portant une charge (10) ayant une ou plusieurs rainures façonnées (18) formées sur la surface (16) et courant le long de la longueur des filaments (10), dans lequel chaque filament (10) contient un matériau polymère électriquement conducteur (14) incorporé sous forme soit d'un mélange soit d'un revêtement qui remplit pratiquement les rainures façonnées (18), dans lequel la section transversale de chaque rainure façonnée (18) présente une forme qui permet un entrecroisement mécanique entre un monofilament (12) et le polymère conducteur (14), ledit milieu pour courroie conducteur ayant des propriétés de dissipation des charges statiques comparables à celles d'un milieu pour courroie à base de métal tout en étant résistant aux bosses et plis, et dans lequel la ou les rainures façonnées (18) permettent une exposition continue du polymère conducteur (14) à la surface du filament (16) lorsque le monofilament (12) s'use de façon que le filament (10) conserve sa conductivité.

2. Milieu pour courroie industriel selon la revendication 1, dans lequel les filaments fonctionnels (10) constituent entre 5 et 100 % de l'étoffe.

3. Milieu pour courroie industriel selon la revendication 1, dans lequel l'étoffe a des propriétés de dissipation des charges statiques des étoffes à base de métal tout en ayant aussi des propriétés physiques comparables à celles d'étoffes synthétiques non conductrices.

4. Milieu pour courroie industriel selon la revendication 3, dans lequel lesdites propriétés physiques comprennent l'un parmi le module, la ténacité, la résistance, l'adhérence, la résistance à l'abrasion, et la durabilité.

5. Milieu pour courroie industriel selon la revendication 1, dans lequel le filament (10) comprend un matériau polymère conducteur (14) mélangé avec des matériaux polymères qui peuvent être orientés.

6. Milieu pour courroie industriel selon la revendication 1, dans lequel le filament (10) est une fibre à deux composants contenant un matériau polymère conducteur (14) et formée par extrusion à l'état fondu.

7. Milieu pour courroie industriel selon la revendication 1, dans lequel le filament (10) comprend une structure orientée revêtue de matériau polymère conducteur (14).

8. Milieu pour courroie industriel selon la revendication 7, dans lequel le polymère conducteur (14) est appliqué par l'un parmi un revêtement par immersion, une pulvérisation à partir de solutions, une dispersion sur le filament, et une pulvérisation thermique.

9. Milieu pour courroie industriel selon la revendication 1, dans lequel le filament (10) comprend un matériau polymère conducteur (14) choisi dans la classe des polyanilines.

10. Milieu pour courroie industriel selon la revendication 9, dans lequel ledit filament de polyaniline a les propriétés physiques d'un filament de polyamide.

11. Milieu pour courroie industriel selon la revendication 1, dans lequel le filament (10) est un monofilament lobé (12) revêtu de matériau polymère conducteur (14).

12. Milieu pour courroie industriel selon la revendication 11, dans lequel le revêtement (14) a une conductivité au minimum supérieure à 10⁻³ S/cm tout en conservant les propriétés physiques et tribologiques du monofilament de coeur (12).

13. Milieu pour courroie industriel selon la revendication 11, dans lequel la forme de la ou des rainures façonnées (18) comprend des rainures en forme de C qui réalisent un entrecroisement mécanique entre le monofilament et le polymère conducteur (14) remplissant les rainures (18).

14. Milieu pour courroie industriel selon la revendication 13, dans lequel l'entrecroisement réalisé par les rainures en forme de C (18) réduit la nécessité d'une adhérence du polymère conducteur (14) au monofilament (12) en réalisant un entrecroisement mécanique entre le monofilament et le polymère conducteur remplissant les rainures (18).

15. Milieu pour courroie industriel selon la revendication 13, dans lequel le positionnement du polymère conducteur (14) dans les rainures en forme de C (18) blinde le polymère et réduit l'impact de sa moindre résistance à l'abrasion et de ses propriétés physiques.

16. Milieu pour courroie industriel selon la revendication 11, dans lequel le pourcentage en poids du matériau conducteur (14) dans la composition est de 10 % ou moins du poids total du monofilament revêtu (12).

17. Milieu pour courroie industriel selon la revendication 1, dans lequel l'étoffe est monocouche ou multicouche ou stratifiée.

18. Milieu pour courroie industriel selon la revendication 1, lequel milieu pour courroie industriel est l'un parmi les réseaux tissés, non-tissés, liés en spirale, à fils MD ou CD, les étoffes tricotées, les treillis extrudés, et les bandes enroulées en spirale de matériaux tissés et non-tissés.

19. Milieu pour courroie industriel selon la revendication 1, dans lequel l'étoffe convient pour une application à sec dans laquelle une dissipation statique est requise pour le milieu à courroie.

20. Milieu pour courroie industriel selon la revendication 1, dans lequel le polymère conducteur (14) est l'un parmi le polyacétylène, le polythiophène, un poly(3-alkylthiophène), le polypyrrole, le polyisothianaphtalène, le poly(éthylène-dioxythiophène), un poly(paraphénylène-vinylène) à substitution alcoxy, le poly(paraphénylène-vinylène), un poly(2,5-dialcoxy-paraphénylène), le poly(para-phénylène), le poly(para-phénylène) du type en échelle, le poly(sulfure de para-phénylène), le polyheptadiyne, et le poly(3-hexylthiophène).

21. Milieu pour courroie industriel selon la revendication 11, dans lequel le revêtement (14) a une conductivité supérieure à 10³ S/cm tout en conservant les propriétés physiques et tribologiques du monofilament de coeur (12).

22. Milieu pour courroie industriel selon la revendication 1, lequel milieu pour courroie industriel est stratifié.

23. Milieu pour courroie industriel selon la revendication 18, dans lequel les bandes enroulées en spirale sont des matériaux tissés ou non-tissés comprenant des fils contenant des monofilaments, des monofilaments retors, des multifilaments, des multifilaments retors, et des fibres discontinues.

24. Milieu pour courroie industriel selon la revendication 1, dans lequel le monofilament (12) a une forme en section transversale non circulaire.

25. Milieu pour courroie industriel selon la revendication 24, dans lequel le monofilament (12) a une forme en coupe transversale non circulaire choisie dans le groupe constitué par les formes : rectangulaire, carrée, trapézoïdale, oblongue, ovale, conique, et en étoile.

26. Milieu pour courroie industriel selon la revendication 25, dans lequel la forme en coupe transversale du monofilament (12) est rectangulaire ou carrée et comprend une pluralité de rainures.

27. Milieu pour courroie industriel selon la revendication 11, dans lequel la forme d'une ou plusieurs rainures façonnées (18) comprend un étranglement qui permet un entrecroisement mécanique entre le monofilament et le polymère conducteur (14) remplissant les rainures (18).

28. Filament polymère portant une charge (10) convenant pour un milieu pour courroie industriel technique destiné à la fabrication de textiles non-tissés selon des procédés pneumatiques air-laid, de fusion-soufflage et/ou de filage-liage, ledit filament polymère (10) ayant une ou plusieurs rainures façonnées (18) formées sur la surface (16) et courant le long de la longueur des filaments (10), dans lequel lesdites rainures façonnées (18) sont pratiquement remplies de matériau polymère électriquement conducteur (14) mécaniquement verrouillé en place, et dans lequel la ou les rainures façonnées (18) permettent une exposition continue du polymère conducteur (14) à la surface du filament (18) lorsque le monofilament (12) s'use de façon que le filament (10) conserve sa conductivité, et dans lequel la section transversale de chaque rainure façonnée (18) présente une forme qui permet un entrecroisement mécanique entre le monofilament (12) et le polymère conducteur (14).

29. Filament selon la revendication 28, lequel filament (10) comprend un matériau polymère conducteur (14) mélangé avec des matériaux polymères qui peuvent être orientés.

30. Filament (10) selon la revendication 28, lequel filament (10) est une fibre à deux composants contenant un matériau polymère conducteur (14) et formée par extrusion à l'état fondu.

31. Filament (10) selon la revendication 28, lequel filament (10) comprend une structure orientée revêtue de matériau polymère conducteur (14).

32. Filament (10) selon la revendication 31, dans lequel le polymère conducteur (14) est appliqué par l'un parmi un revêtement par immersion, une pulvérisation à partir de solutions, une dispersion sur le filament, et une pulvérisation thermique.

33. Filament (10) selon la revendication 28, lequel filament comprend un matériau polymère conducteur (14) choisi dans la classe des polyanilines.

34. Filament (10) selon la revendication 33, dans lequel ledit filament de polyaniline a les propriétés physiques d'un filament de polyamide.

35. Filament (10) selon la revendication 28, lequel filament est un monofilament lobé (12) revêtu de matériau polymère conducteur (14).

36. Filament (10) selon la revendication 35, dans lequel le revêtement (14) a une conductivité au minimum supérieure à 10³ S/cm tout en conservant les propriétés physiques et tribologiques du monofilament de coeur.

37. Filament (10) selon la revendication 35, dans lequel la forme de la ou des rainures façonnées (18) comprend des rainures en forme de C qui réalise un entrecroisement mécanique entre le monofilament (12) et le polymère conducteur (14) remplissant les rainures (18).

38. Filament (10) selon la revendication 37, dans lequel l'entrecroisement réalisé par les rainures en forme de C (18) réduit la nécessité d'une adhérence du polymère conducteur (14) au monofilament (12) en réalisant un entrecroisement mécanique entre le monofilament (12) et le polymère conducteur (14) remplissant les rainures (18).

39. Filament (10) selon la revendication 37, dans lequel le positionnement du polymère conducteur (14) dans les rainures en forme de C (18) blinde le polymère (14) et réduit l'impact de sa moindre résistance à l'abrasion et de ses propriétés physiques.

40. Filament (10) selon la revendication 35, dans lequel le pourcentage en poids du matériau conducteur (14) dans la composition est de 10 % ou moins du poids total du monofilament revêtu (12).

41. Filament (10) selon la revendication 28, dans lequel le polymère conducteur (14) est l'un parmi le polyacétylène, le polythiophène, un poly(3-alkylthiophène), le polypyrrole, le polyisothianaphtalène, le poly(éthylène-dioxythiophène), un poly(paraphénylène-vinylène) à substitution alcoxy, le poly(paraphénylène-vinylène), un poly(2,5-dialcoxyparaphénylène), le poly(para-phénylène), le poly(para-phénylène) du type en échelle, le poly(sulfure de para-phénylène), le polyheptadiyne, et le poly(3-hexylthiophène).

42. Filament (10) selon la revendication 35, dans lequel le revêtement (14) a une conductivité supérieure à 10³ S/cm tout en conservant les propriétés physiques et tribologiques du monofilament de coeur.

43. Filament (10) selon la revendication 28, dans lequel le monofilament (12) a une forme en section transversale non circulaire.

44. Filament selon la revendication 43, dans lequel le monofilament (12) a une forme en coupe transversale non circulaire choisie dans le groupe constitué par les formels : rectangulaire, carrée, trapézoïdale, oblongue, ovale, conique, et en étoile.

45. Filament (10) selon la revendication 44, dans lequel la forme en coupe transversale non circulaire du monofilament (12) est rectangulaire ou carrée et comprend une pluralité de rainures.

46. Filament (10) selon la revendication 21, dans lequel la forme de la ou des rainures façonnées (18) comprend un étranglement qui permet un entrecroisement mécanique entre le monofilament et le polymère conducteur (14) remplissant les rainures (18).
